

## UNITED STATES PATENT OFFICE

2,599,178

ELECTRODEPOSITION OF ALLOYS OF  
MOLYBDENUM WITH COBALT, NICKEL,  
AND IRON

Matthew L. Holt, Madison, Wis., and Henry J. Seim, Reno, Nev., assignors to Wisconsin Alumni Research Foundation, Madison, Wis., a corporation of Wisconsin

No Drawing. Application March 10, 1950,  
Serial No. 149,022

14 Claims. (Cl. 204—43)

**1** This invention relates, generally, to the electrodeposition of molybdenum alloys and it has particular relation to the electrodeposition of alloys of molybdenum with cobalt, nickel or iron.

Among the objects of this invention are: To provide for the electrodeposition of alloys of molybdenum with cobalt, nickel and iron; to improve the current efficiency in the electrodeposition process; to increase the molybdenum content of the alloy deposited on the cathode; and to provide a new bath for use in accomplishing these objects.

The plating bath in accordance with the invention contains an organic hydroxy acid or complexing agent, such as citric acid, tartaric acid and glycolic acid, a soluble molybdate, such as sodium molybdate and ammonium molybdate, a compound of the alloying metal (cobalt, nickel or iron), such as the sulfate, ammonium hydroxide and water. Electrolysis of this plating bath using soluble anodes, such as cobalt, nickel, iron, or molybdenum anodes, or an insoluble anode, such as platinum, effects the deposition of an alloy of molybdenum with the alloying metal (cobalt, nickel or iron) on the cathode. The cathode may be formed of any suitable material such as platinum, gold, copper, iron, nickel, cobalt, brass, or other metals or alloys. While the temperature of the plating bath may vary from room temperature to the boiling point of the solution, best results are obtained when it is kept at a temperature of from 20 to 30° C. There appears to be no critical cathode current density for the plating bath. The optimum current density is dependent on other electrolysis conditions and the composition of the bath. Cathode current densities that have been found to be satisfactory vary from about 1 ampere per square decimeter to 22.2 amperes per square decimeter.

Experimental work in connection with this invention shows that the concentration of the alloying metal compound in the plating bath is not critical. However, it was found that the amount of complexing agent, citric acid in accordance with this invention, which is required depends upon the amount of alloying metal compound which is present. While the amount of the complexing agent is not critical, it appears that, when citric acid is employed, a slight excess of it over the amount of alloying metal compound is re-

quired. Preferably a ratio of about 1.5 moles of citric acid to one mole of the alloying metal is employed.

The amount of the soluble molybdate compound which is used to provide a good alloy deposit on the cathode varies according to the electrolysis conditions. In accordance with this invention sodium molybdate is employed. Satisfactory alloy deposits have been obtained from 5 baths of the present invention containing less than two grams per liter and as much as forty grams per liter of sodium molybdate. The use of four grams of sodium molybdate per liter gives excellent results.

15 In order to obtain satisfactory alloy deposits on the cathode it is necessary to control the pH of the plating bath. While alloy deposits of molybdenum can be obtained from plating baths of the present invention with a range of pH from 20 three to nine, it appears, in general, when the bath is neutral or basic (pH 7 to 9), higher cathode current densities are required. For the cobalt-molybdenum bath, a pH of 4 appears to be most satisfactory. For the nickel-molybdenum 25 bath, a pH of either four or eight is satisfactory. For the iron-molybdenum bath, a pH of six was found to give optimum results. In accordance with this invention ammonium hydroxide is employed for adjusting the pH of the bath.

30 The amount of molybdenum present in the alloy deposit on the cathode is dependent on the electrolysis conditions and the composition of the bath. In general, the highest percentage of molybdenum (50% or more) was obtained with 35 iron as the alloying metal. The lowest percentage of molybdenum was obtained when nickel was used as the alloying metal.

The following baths are typical of those which 40 can be used to give satisfactory molybdenum alloy deposits.

## Cobalt-molybdenum plating bath

|                                            |       |    |
|--------------------------------------------|-------|----|
| Cobalt sulfate heptahydrate                | grams | 60 |
| 45 Citric acid                             | do    | 66 |
| Sodium molybdate                           | do    | 4  |
| Ammonium hydroxide sufficient to provide a |       |    |
| 50 pH of 4                                 |       |    |
| Water to give a total volume of 1 liter    |       |    |
| 50 Temperature of 25° C.                   |       |    |

With the cobalt-molybdenum bath adjusted to a pH of 4, electrolysis at ten amperes per square decimeter deposited a cobalt-molybdenum alloy on the cathode containing 6.9 per cent molybdenum with a cathode current efficiency of 36 per cent. When the pH of the bath was increased to six, electrolysis at the same current density deposited an alloy on the cathode containing 27.2 per cent molybdenum at a cathode current efficiency of 40 per cent.

*Nickel-molybdenum plating bath*

|                                                          |       |    |
|----------------------------------------------------------|-------|----|
| Nickel sulfate hexahydrate                               | grams | 60 |
| Citric acid                                              | do    | 66 |
| Sodium molybdate                                         | do    | 4  |
| Ammonium hydroxide sufficient to provide the required pH |       |    |
| Water to give a total volume of 1 liter                  |       |    |
| Temperature of 25° C.                                    |       |    |

With a bath pH of 4 and a current density of ten amperes per square decimeter, the nickel molybdenum alloy deposit on the cathode contained 13 per cent molybdenum and the cathode current efficiency was 24 per cent. When the pH of the bath was increased to 8, electrolysis at this same current density deposited an alloy on the cathode containing 15.8 per cent molybdenum with a cathode current efficiency of 62 per cent.

*Iron-molybdenum plating bath*

|                                                          |       |    |
|----------------------------------------------------------|-------|----|
| Ferrous sulfate heptahydrate                             | grams | 60 |
| Citric acid                                              | do    | 66 |
| Sodium molybdate                                         | do    | 4  |
| Ammonium hydroxide sufficient to provide the required pH |       |    |
| Water to give a total volume of 1 liter                  |       |    |
| Temperature of 25° C.                                    |       |    |

When the pH of the bath was adjusted to 6, electrolysis at 10 amperes per square decimeter deposited an alloy on the cathode containing 48.6 per cent molybdenum at a cathode current efficiency of 17 per cent. On increasing the pH of the bath to 7, electrolysis at the same current density deposited an alloy containing 62 per cent molybdenum with a current efficiency of 13 per cent.

What is claimed as new is:

1. Method of electrodepositing an alloy of molybdenum and a metal of the class consisting of cobalt, nickel and iron which comprises: passing current between an anode and a cathode on which the alloy is to be deposited in an aqueous electrolyte consisting essentially of 60 grams per liter of a sulfate selected from the class consisting of cobalt, nickel and iron, citric acid in an amount in excess of the sulfate, 2 to 40 grams per liter of sodium molybdate, and sufficient ammonium hydroxide to provide a pH of from 4 to 8.

2. The invention, as set forth in claim 1, wherein 1.5 moles of citric acid are used to one mole of sulfate.

3. The invention, as set forth in claim 2, wherein the cathode current density ranges from 1 to 22.2 amperes per square decimeter.

4. Method of electrodepositing an alloy of molybdenum and a metal of the class consisting of cobalt, nickel and iron which comprises: passing current between an anode and a cathode on which the alloy is to be deposited in an aqueous electrolyte consisting essentially of 60 grams per liter of a sulfate selected from the class consisting of cobalt, nickel and iron, 66 grams per liter of citric acid, 4 grams per liter of sodium molyb-

date, and sufficient ammonium hydroxide to provide a pH ranging from 4 to 8.

5. The invention, as set forth in claim 4, wherein the cathode current density ranges from 1 to 22.2 amperes per square decimeter.

6. A bath for electrodepositing an alloy of molybdenum and a metal of the class consisting of cobalt, nickel and iron consisting essentially of an aqueous electrolyte containing 60 grams per liter of a sulfate selected from the class consisting of cobalt, nickel and iron, citric acid in an amount in excess of the sulfate, 2 to 40 grams per liter of sodium molybdate, and sufficient ammonium hydroxide to provide a pH of from 4 to 8.

7. The invention, as set forth in claim 6, wherein 1.5 moles of citric acid are used to one mole of sulfate.

8. A bath for electrodepositing an alloy of molybdenum and a metal of the class consisting of cobalt, nickel and iron consisting essentially of an aqueous electrolyte containing 60 grams per liter of a sulfate selected from the class consisting of cobalt, nickel and iron, 66 grams per liter of citric acid, 4 grams per liter of sodium molybdate, and sufficient ammonium hydroxide to provide a pH of from 4 to 8.

9. A bath for electrodepositing an alloy of molybdenum and a metal of the class consisting of cobalt, nickel and iron consisting essentially of:

|                                                                       |       |    |
|-----------------------------------------------------------------------|-------|----|
| Sulfate selected from the class consisting of cobalt, nickel and iron | grams | 60 |
| Citric acid                                                           | do    | 66 |
| Sodium molybdate                                                      | do    | 4  |
| Ammonium hydroxide sufficient to provide a pH ranging from 4 to 8.    |       |    |
| Water to give a volume of 1 liter.                                    |       |    |

10. A bath for electrodepositing an alloy of molybdenum and cobalt consisting essentially of:

|                                                     |       |    |
|-----------------------------------------------------|-------|----|
| Cobalt sulfate heptahydrate                         | grams | 60 |
| Citric acid                                         | do    | 66 |
| Sodium molybdate                                    | do    | 4  |
| Ammonium hydroxide sufficient to provide a pH of 4. |       |    |
| Water to give a volume of 1 liter.                  |       |    |

11. A bath for electrodepositing an alloy of molybdenum and cobalt consisting essentially of:

|                                                     |       |    |
|-----------------------------------------------------|-------|----|
| Cobalt sulfate heptahydrate                         | grams | 60 |
| Citric acid                                         | do    | 66 |
| Sodium molybdate                                    | do    | 4  |
| Ammonium hydroxide sufficient to provide a pH of 6. |       |    |
| Water to give a volume of 1 liter.                  |       |    |

12. A bath for electrodepositing an alloy of molybdenum and nickel consisting essentially of:

|                                                     |       |    |
|-----------------------------------------------------|-------|----|
| Nickel sulfate hexahydrate                          | grams | 60 |
| Citric acid                                         | do    | 66 |
| Sodium molybdate                                    | do    | 4  |
| Ammonium hydroxide sufficient to provide a pH of 4. |       |    |
| Water to give a volume of 1 liter.                  |       |    |

13. A bath for electrodepositing an alloy of molybdenum and nickel consisting essentially of:

|                                                     |       |    |
|-----------------------------------------------------|-------|----|
| Nickel sulfate hexahydrate                          | grams | 60 |
| Citric acid                                         | do    | 66 |
| Sodium molybdate                                    | do    | 4  |
| Ammonium hydroxide sufficient to provide a pH of 8. |       |    |
| Water to give a volume of 1 liter.                  |       |    |

14. A bath for electrodepositing an alloy of molybdenum and iron consisting essentially of:

Ferrous sulfate heptahydrate \_\_\_\_\_ grams 60

Citric acid \_\_\_\_\_ do 66

Sodium molybdate \_\_\_\_\_ do 4 5

Ammonium hydroxide sufficient to provide a pH of 6.

Water to give a volume of 1 liter.

MATTHEW L. HOLT. 10

HENRY J. SEIM.

## REFERENCES CITED

The following references are of record in the file of this patent:

## UNITED STATES PATENTS

| Number    | Name             | Date         |
|-----------|------------------|--------------|
| 2,160,322 | Armstrong et al. | May 30, 1939 |
| 2,428,404 | Yntema           | Oct. 7, 1947 |

## OTHER REFERENCES

Metal Industry, Nov. 22, 1946, pp. 434, 435, 436  
(an article by L. E. Valler and M. L. Holt).